

# UNITED STATES PATENT OFFICE.

GEORGE O. SEWARD AND FRANZ VON KÜGELGEN, OF HOLCOMBS ROCK, VIRGINIA, ASSIGNORS  
TO VIRGINIA LABORATORY COMPANY, OF NEW YORK, N. Y., A CORPORATION OF NEW  
YORK.

## PRODUCTION OF MAGNESIUM BY ELECTROLYSIS.

No. 900,961.

Specification of Letters Patent.

Patented Oct. 13, 1908.

Application filed October 10, 1905. Serial No. 282,113.

*To all whom it may concern:*

Be it known that we, GEORGE O. SEWARD, a citizen of the United States, and FRANZ VON KÜGELGEN, a subject of the German Empire, both residing at Holcombs Rock, in the county of Bedford and State of Virginia, have jointly invented certain new and useful Improvements in the Production of Magnesium by Electrolysis, of which the following is a specification.

When the attempt is made to produce magnesium by electrolyzing a mixture of magnesium fluorid and an alkali chlorid, it is always found that the separated magnesium contains injurious quantities of the alkali metal. Even with a high concentration of  $MgF_2$ , this is the case. The explanation is as follows:—The alkali chlorid, having a lower decomposition voltage than  $MgF_2$ , is separated first. The  $MgF_2$  is then reduced by the nascent alkali metal in a secondary reaction. This reaction is, however, not complete, and a portion of the alkali metal alloys with the magnesium.

According to the present invention the above difficulties are avoided by using, instead of the alkali chlorid, an earth alkali chlorid of a more electropositive metal than magnesium (in which term we include one or more such chlorids), which is decomposed electrolytically only with difficulty. A pure magnesium is then obtained. For example,  $MgF_2$  and  $CaCl_2$  are mixed and melted, and then heated until all water is driven out. The addition of a small percentage of an alkali fluorid as a flux assists in this operation. The resulting molten mixture is electrolyzed, and we obtain magnesium at the cathode and chlorin at the anode, the  $CaCl_2$  having been changed to the fluorid.

When the electrolyte becomes too poor in magnesium, it is worked over as follows:—It is mixed with fused hydrated  $MgCl_2$ , and heated until all water is driven out. The magnesium chlorid and calcium fluorid ( $MgCl_2 + CaF_2$ ) change to magnesium fluorid and calcium chlorid ( $MgF_2 + CaCl_2$ ).

Though we have described with great particularity of detail certain specific processes

embodimenting the invention, yet it is not to be understood therefrom that the invention is limited to the specific embodiments described.

Various modifications may be made by those skilled in the art without departure from the invention.

What we claim is:—

1. The process of producing magnesium, which consists in fusing together magnesium-fluorid and calcium chlorid, with a flux of an alkali fluorid, heating to render the bath anhydrous, then electrolyzing to produce magnesium, the calcium chlorid being changed to calcium fluorid, and reconstituting the bath by adding hydrated magnesium chlorid and heating to dehydrate it, whereby the calcium fluorid and magnesium chlorid react to form magnesium fluorid and calcium chlorid, and resuming the electrolysis.

2. The process of producing magnesium, which consists in electrolyzing a fused mixture of magnesium fluorid and a chlorid of an earth-alkali metal more electro-positive than magnesium.

3. The process of producing magnesium, which consists in electrolyzing a fused mixture of magnesium fluorid and a chlorid of an earth-alkali metal more electro-positive than magnesium, and renewing the magnesium content of the electrolyte by the addition of a magnesium salt.

4. The process of producing magnesium, which consists in electrolyzing a fused mixture of magnesium fluorid and a chlorid of an earth-alkali metal more electro-positive than magnesium, with a small percentage of an alkali fluorid as a flux.

5. The process of producing magnesium, which consists in electrolyzing a fused mixture of magnesium fluorid and an earth-alkali-chlorid of a more electro-positive metal than magnesium, and renewing the magnesium content of the electrolyte by addition of magnesium chlorid, which reacts with the earth-alkali fluorid produced by the electrolysis, to form magnesium fluorid.

6. The process of producing magnesium, which consists in electrolyzing a fused mix-

ture of magnesium fluorid and a chlorid of an earth-alkali metal more electro-positive than magnesium, and renewing the magnesium content of the electrolyte by addition of fused hydrated magnesium chlorid, heating to expel the water, and subjecting it again to electrolysis.

In witness whereof, we have hereunto

signed our names in the presence of two subscribing witnesses.

GEORGE O. SEWARD.  
FRANZ VON KÜGELGEN.

Witnesses:

DOMINGO A. USINA,  
THEODORE T. SNELL.